

## 1

3,378,581

## DIAMINE SALTS USEFUL FOR INHIBITING THE CORROSION IN RETURN STEAM CONDENSATE LINES

Louis E. Hummel, East View, San Pedro, Calif., assignor to Nalco Chemical Company, Chicago, Ill., a corporation of Delaware

No Drawing. Original application May 10, 1956, Ser. No. 583,397, now Patent No. 3,029,125, dated Apr. 10, 1962. Divided and this application July 31, 1961, Ser. No. 127,821

4 Claims. (Cl. 260—501,17)

The subject application is a divisional application of my copending application Ser. No. 583,397 which was filed on May 10, 1956.

This invention relates to novel compounds which are useful in inhibiting corrosion in return steam condensate lines. More particularly, the subject invention is directed to new compositions of matter which are organic acid salts of the reaction product of an alkylene oxide and a substituted alkylene diamine.

It is well known that steam lines and steam condensate lines are subject to corrosion which is very difficult to control. This corrosion is apparently due, to a large extent, to carbon dioxide and oxygen in the boiler-steam-condensate system. Carryover from the boiler water can also increase the corrosion. The problem of corrosion of the internal surfaces of steam condensate return lines has been recognized for many years. Generally, the difficulties that have been experienced are pitting, grooving and ultimate deterioration of sections of the condensate return system and the plugging of constrictions in the system with the insoluble products of corrosion. To evaluate properly the actual cost of return line corrosion, it is necessary not only to consider the loss in terms of labor, curtailed production and the cost of the material destroyed, but also to weigh effects in terms of inefficient operation of fouled equipment.

Experimental studies by various investigators indicate that dissolved carbon dioxide and oxygen are responsible for practically all the corrosion in the condensate lines. The various expedients that have been devised for combating this attack are as follows:

(1) The use of corrosion resistant alloys, which is generally prohibitive from a cost standpoint.

(2) Minimizing the amount of carbon dioxide and oxygen in the condensate either by venting or pretreatment of the boiler feedwater.

(3) Chemical treatment of the condensate.

It is known to use a readily volatile alkaline amine material for protection against corrosion in steam and return condensate lines but the results obtained with such amines have sometimes left much to be desired, particularly in steam and condensate systems of great length or in tall buildings. Moreover, these amines to be effective, are usually required in amounts which are roughly proportional to the carbon dioxide content of the condensate. Where the return of condensate to the boiler constitutes a minor fraction of the boiler feed, such treatment often becomes economically impractical.

Where high pressure steam is required to operate industrial devices, such as turbines, it has been the experience of the art that certain treating agents will undergo decomposition and form deposits on the surfaces of the devices which, in many instances, will necessitate costly shutdowns and repairs.

It would be desirable to have a chemical treatment capable of being applied to any part of a steam or condensate return system at small, economical dosages and have beneficial results obtained in all cases.

The principal object of the present invention is to provide compositions of matter for the treatment of steam

## 2

condensates which produce improved results in preventing or minimizing corrosion in steam lines, traps, condensers, valves, and in other parts of steam systems such as turbine blades.

It has been found that the corrosion in steam and condensate return systems may be prevented or substantially mitigated by treating such systems with a corrosion inhibiting amount of a carboxylic acid salt of the reaction product of a low molecular weight alkylene oxide and a substituted alkylene diamine. These materials are effective when added either to the boiler feedwater, to the steam lines, or to the condensate return lines. When added to the boiler feedwater it is generally necessary to add a slightly excessive amount to insure that enough of the chemical steam distills into the steam and condensate return systems. Generally, however, it is preferred to add the treatment to the steam condensate line since it is this part of the system where corrosive attack is the severest and the smallest amounts of the treatment are the most effective. From a practical standpoint, the chemical is most conveniently applied to the boiler feedwater.

The amount of treatment should be at least 1 part per million of the corrosion inhibiting chemical by weight of the steam or steam condensate, preferably 2 to 5 parts per million and even more preferably 10 to 25 parts per million. The dosage will, of course, vary depending on the conditions of the system and other variable factors and hence, dosages as high as 50 to 100 parts per million may be necessary under extraordinarily corrosive conditions.

The employment of the corrosion inhibiting chemicals in accordance with this invention is applicable to the generation of steam at various temperatures and pressures. Good results can be obtained where steam is generated under atmospheric conditions, subatmospheric conditions or superatmospheric conditions. In most cases, steam is generated at pressures from atmospheric up to 1500 pounds per square inch or more and the corresponding temperatures.

The substituted alkylene diamines which are used as starting materials in preparing the compositions useful in the practice of the invention have the following general formula:



wherein R is an acyclic hydrocarbon radical containing from 10 to 32 carbon atoms and n is an integer from 2 to 6.

The radical R is conveniently derived from a saturated or unsaturated fatty group. Such groups as dodecyl, tetradecyl, hexadecyl, octadecyl, octadecenyl, and octadecadienyl may be substituents with good results being obtained in each instance. Extremely good results are afforded when R is a mixture of alkyl radicals such as are found in vegetable oils and animal fats. Coco, soya and tallow are examples of such mixed natural radicals.

The diamine portion of the compounds described above may be one of any number of the known diamines. Ethylene diamine, 1,2 - propylene diamine, 1,3 - propylene diamine and hexamethylene diamine are several examples.

The substituted alkylene diamines may be prepared by several different techniques. For instance, the alkylene diamines may be alkylated with an alkyl halide to produce the desired product. Such a method is illustrated in Kyrides U.S. Patent 2,246,524. Another method is to react an alkylamine with acrylonitrile and then hydrogenate whereby an alkyl substituted propylene diamine is produced. Commercially available N-alkyl propylene diamines are the products manufactured by the Armour Chemical Division under the trade name, "Duomeens."

Specific Duomeens are N-lauryl propylene diamine; N-coco propylene diamine; N-soya propylene diamine, and N-tallow propylene diamine.

The substituted alkylene diamines thus described are capable of being reacted with varying amounts of several of the well known low molecular weight alkylene oxides, such as ethylene oxide, 1,2-propylene oxide, butylene oxide or the like, to produce products varying in their physical and chemical properties. To be suitable for present purposes, the hydroxyalkylated, substituted alkylene diamines must be water dispersible to the extent that 5% by weight or more forms a uniform dispersion in aqueous media. This is usually accomplished by hydroxyalkylating 1 mol of diamine with 1 to 4, and preferably 2-3, mols of ethylene oxide or other alkylene oxide to produce the degree of water dispersibility desired.

The hydroxyalkylation of the products may be performed by any one of several well known methods. Since there are three reactive hydrogen atoms in the alkyl substituted diamines the hydroxyalkylation could conceivably take place at any of the sites. Hence, one mol of an alkylene oxide could react with any one of the three hydrogen atoms to produce a mixture of hydroxyalkylated products. Several of these reaction products are listed below in Table I.

TABLE I

| Composition Number | Alkyl Substituted Propylene Diamine | Mols of Ethylene Oxide | Water Dispersible |    |
|--------------------|-------------------------------------|------------------------|-------------------|----|
|                    |                                     |                        | Yes               | No |
| I                  | N-tallow propylene diamine          | 3                      | X                 |    |
| II                 | do                                  | 2                      | X                 |    |
| III                | do                                  | 1                      | X                 |    |
| IV                 | N-soya propylene diamine            | 3                      | X                 |    |
| V                  | N-coco propylene diamine            | 3                      | X                 |    |
| VI                 | N-lauryl propylene diamine          | 4                      | X                 |    |
| VII                | N-coco propylene diamine            | 2                      | X                 |    |

The salt forming aliphatic carboxylic acids should not exceed 10 carbon atoms in chain length. For purpose of classification the acids may be divided into four classes:

- (I) Aliphatic monocarboxylic acids
- (II) Aliphatic dicarboxylic acids
- (III) Hydroxy substituted carboxylic acids
- (IV) Hydroxy substituted polycarboxylic acids

In class I such acids as acetic, propionic, n-butyric, isobutyric, n-heptylic, caprylic and prelarnic acids may be used. Examples of class II are oxalic, malonic, succinic, glutaric, adipic, pimelic, suberic, azelaic and sebacic acids. Glycolic, gluconic, glyceric and lactic acids are illustrative of class III. Class IV would include such acids as malic and citric.

For purposes of illustration, several aliphatic carboxylic acid salts of the alkyl substituted propylene diamines listed in Table I are shown below in Table II.

TABLE II

| Composition Number | Composition Number<br>Table I | Aliphatic Carboxylic Acid | Mol Ratio<br>Reaction Product:Acid |
|--------------------|-------------------------------|---------------------------|------------------------------------|
| VIII               | I                             | Acetic acid               | 1:1                                |
| IX                 | I                             | Lactic acid               | 1:1                                |
| X                  | I                             | Citric acid               | 1:1                                |
| XI                 | III                           | Butyric acid              | 1:1                                |
| XII                | IV                            | Malic acid                | 1:1                                |
| XIII               | V                             | Succinic acid             | 1:1                                |
| XIV                | I                             | Malonic acid              | 2:1                                |
| XV                 | I                             | Adipic acid               | 1:1                                |

The salts listed in Table II were prepared by heating the compositions in Table I, which ranged from viscous liquids to pastes, and adding the acid, with continued heat, until a homogeneous product was produced.

When boiler feedwater applications are contemplated it is sometimes helpful to formulate the compositions of the invention with boiler antifoams. The compositions of the invention will not produce foaming or priming when used at the concentrations recommended herein, but in

the event high concentrations occur in the boiler water, the use of antifoams is a safeguard to insure good operation of the boiler. Antifoams that may be used are those described in U.S. Patents 2,575,298, 2,626,243, 2,575,276, 2,609,344 and 2,717,881. Only a few parts per million of these antifoams in the boiler water are required to insure against any harmful foaming.

#### EVALUATION OF THE INVENTION

(A) Screening tests.—The material to be tested was added, at a concentration of 100 parts per million, to 350 ml. of deionized water contained in a 400 ml. beaker. The beaker was held in an oil bath at a temperature of about 145° F. The solution was stirred at about 1750 r.p.m. with centrifugal-type glass stirrers. A mixture of CO<sub>2</sub> and air was bubbled through the solution during the test. A mild steel specimen was sandblasted, weighed, and placed in the solution overnight. The weight loss of the specimen was then determined. A similar test, called the blank, was made under identical conditions except that no corrosion inhibitor was added to the water. The data from these screening tests are presented in Table III as percent protection compared with the blank test.

TABLE III

| Composition              | Percent protection       |    |
|--------------------------|--------------------------|----|
|                          | Composition IX, Table II | 93 |
| Sebacic acid             |                          | 11 |
| Sodium hexametaphosphate |                          | 19 |
| Octadecyl urea           |                          | 0  |

From the above it is evident the compositions of the invention provided superior corrosion protection as against the poor or slight protection afforded by other inhibitors tested.

(B) Experimental condensate corrosion tests.—This series of corrosion tests were made in an apparatus designed to simulate a severely corrosive condition which might be encountered in a steam condensate system. In this apparatus a synthetic condensate was produced in a glass tower by aerating heated distilled water with a mixture of carbon dioxide and air. This condensate and a solution of the treating chemical were proportioned into a test container by gravity feed. A number of steel test coupons were suspended in the latter and the liquid was mildly agitated with a paddle stirrer. At periodic intervals a test specimen was removed from the bath and the weight loss determined. The temperature, free carbon dioxide and dissolved oxygen of the synthetic condensate, and the treatment concentration were controlled throughout the test.

The corrosion test specimens consisted of 1 inch x 2 inch panels which were sheared from a single sheet of 22 gauge cold rolled mild steel. All specimens were uniformly sandblasted before being immersed in the bath.

Agitation of the liquid was initiated and the water in the bath was heated to and thermostatically controlled at 150° ± 1° F. The free carbon dioxide and dissolved oxygen of the water were maintained at 45 ± 4 parts per million and 3.5 ± 0.2 parts per million, respectively.

A complete, detailed description of the test apparatus and method is described in the article, "A Laboratory Method for the Study of Steam Condensate Corrosion Inhibitors," by H. I. Patzelt, Corrosion, January 1953.

The following examples illustrate the results obtained in the evaluation of test specimens using treating chemicals within the scope of the invention.

#### Example I

In this series the two compositions, composition VIII, Table II and composition IX, Table II were each tested separately at 10 parts per million. At the end of the 6th day the weight losses were 221 and 121 milligrams, respectively.

The corrosive conditions maintained in these tests when

compared with most industrial condensate return systems are extremely severe. Inhibitors giving only good to fair results in the test in most cases give outstanding results in actual use at lower dosages.

(C) Effect on brass.—The screening test method (A above) was used. Brass specimens in place of the steel were suspended in deionized water. Rather than running a percent comparison against the blank, weight losses in milligrams were determined. Composition XVI showed a weight loss of only 13.2 milligrams.

#### Example II

This test was conducted in an actual boiler system to determine whether composition XVI would be detrimental to normal boiler operation. The test boiler generated a total of 800,000 to 1,000,000 pounds of steam per day at 125 pounds per inch. Composition XVI was fed by dispersing 1 gallon into 30 to 40 gallons of condensate return and injecting it directly into the steam header. The dosage for the entire test period was maintained at 10 parts per million of the steam.

A by-pass corrosion test loop was installed in front of one of the condensate return pumps. This loop was approximately 3,000 feet from the boiler and 400 to 700 gallons passed through per day. The specimen was a 1 inch pipe nipple which was placed in the system with appropriate fittings.

The test was run for one month at the end of which time inspection revealed corrosion rates of the specimen were being satisfactorily controlled. A sample of condensate was collected from the by-pass loop and analysis showed it to contain  $2.0 \pm 0.6$  parts per million of composition XVI. Of interest is the fact that the sample thus taken was at a point most remote from the boiler. There was no evidence of deposits forming in the system and no unusual foaming occurred in the boiler.

The expression "water dispersible" as used herein means a material which in water or other aqueous media does not form a true solution yet it is capable of remaining in a suspended condition at the concentrations herein specified for relatively long periods of time. These suspensions may or may not be colloidal.

I claim:

1. Salts of an aliphatic carboxylic acid and salts of the reaction product of 3 mols of ethylene oxide per mol of a substituted alkylene diamine of the formula



wherein R is a long chain acyclic hydrocarbon radical containing 10 to 32 carbon atoms, the salt forming aliphatic carboxylic acid being selected from the group consisting of acetic, propionic, n-butyric, isobutyric, n-heptylic, caprylic, pelargonic, oxalic, malonic, succinic, glutaric, adipic, pimelic, suberic, azelaic, sebatic, glycolic, gluconic, glyceric, lactic, malic and citric.

5 2. The acetic acid salt of the reaction product of ethylene oxide and N-tallow propylene diamine in a mol ratio of about 3 mols of ethylene oxide per mol of said diamine.

15 3. The lactic acid salt of the reaction product of ethylene oxide and N-tallow propylene diamine in a mol ratio of about 3 mols of ethylene oxide per mol of said diamine.

20 4. The citric acid salt of the reaction product of ethylene oxide and N-tallow propylene diamine in a mol ratio of about 3 mols of ethylene oxide per mol of said diamine.

#### References Cited

##### UNITED STATES PATENTS

|           |         |              |       |           |
|-----------|---------|--------------|-------|-----------|
| 2,243,329 | 5/1941  | De Groot     | ----- | 260—583   |
| 2,701,239 | 2/1955  | Ryznar       | ----- | 260—584   |
| 2,739,980 | 3/1956  | Chester      | ----- | 260—501   |
| 2,759,021 | 8/1956  | Gaar et al.  | ----- | 260—584   |
| 2,920,040 | 1/1960  | Jolly        | ----- | 260—501   |
| 2,552,531 | 5/1951  | De Groot     | ----- | 260—501   |
| 2,868,833 | 1/1959  | Szabo et al. | ----- | 260—501   |
| 2,914,557 | 11/1959 | Oxford       | ----- | 260—501   |
| 2,995,603 | 8/1961  | Hutchison    | ----- | 260—501   |
| 3,029,125 | 4/1962  | Hummel       | ----- | 21—2.7    |
| 2,143,388 | 1/1939  | Schlock      | ----- | 260—501   |
| 2,736,658 | 2/1956  | Pfohl et al. | ----- | 260—501   |
| 2,952,707 | 9/1960  | Nikawitz     | ----- | 260—501 X |
| 2,930,761 | 3/1960  | Charret      | ----- | 260—584 X |

#### OTHER REFERENCES

Industrial and Engineering Chemistry, vol. 41, No. 10, October 1949, pp. 2080—2090.

LEON ZITVER, Examiner.

LORRAINE A. WEINBERGER, Primary Examiner.

M. B. WEBSTER, B. EISEN, Assistant Examiners.

UNITED STATES PATENT OFFICE  
CERTIFICATE OF CORRECTION

Patent No. 3,378,581

April 16, 1968

Louis E. Hummel

It is certified that error appears in the above identified patent and that said Letters Patent are hereby corrected as shown below:

Column 3, line 46, "prelargonic" should read -- pelargonic --. Column 5, line 44, after "and" cancel "salts". Column 6, line 34, "Schlock" should read -- Schlack --.

Signed and sealed this 25th day of November 1969.

(SEAL)

Attest:

Edward M. Fletcher, Jr.  
Attesting Officer

WILLIAM E. SCHUYLER, JR.  
Commissioner of Patents